

April 7, 1942.

A. M. TALBOT ET AL

2,279,079

HEAT TREATED AND HARDENED ARTICLE OF MANUFACTURE

MADE OF FINE GRAINED DEEP HARDENED STEELS

Filed May 1, 1939

3 Sheets-Sheet 1

*Fig. 1.*



*Fig. 2.*



INVENTORS  
ALBERT M. TALBOT  
WILLIAM C. MEARN

BY

*A. G. Weller*  
ATTORNEY

April 7, 1942.

A. M. TALBOT ET AL

2,279,079

HEAT TREATED AND HARDENED ARTICLE OF MANUFACTURE  
MADE OF FINE GRAINED DEEP HARDENED STEELS

Filed May 1, 1939

3 Sheets-Sheet 2

*Fig. 3.*



*Fig. 4.*



INVENTORS  
ALBERT M. TALBOT  
WILLIAM C. MEARNS  
BY  
A. M. TALBOT  
ATTORNEY

April 7, 1942.

A. M. TALBOT ET AL

2,279,079

HEAT TREATED AND HARDENED ARTICLE OF MANUFACTURE  
MADE OF FINE GRAINED DEEP HARDENED STEELS

Filed May 1, 1939

3 Sheets-Sheet 3

*Fig. 5.*



*Fig. 6.*



INVENTORS  
ALBERT M. TALBOT  
WILLIAM C. MEARNS  
BY

*A. M. Talbot*  
ATTORNEY

## UNITED STATES PATENT OFFICE

2,279,079

HEAT TREATED AND HARDENED ARTICLE  
OF MANUFACTURE MADE OF FINE  
GRAINED DEEP HARDENED STEELS

Albert M. Talbot, Fair Haven, and William C. Mearns, Elizabeth, N. J., assignor to The International Nickel Company, Inc., New York, N. Y., a corporation of Delaware

Application May 1, 1939, Serial No. 270,992

4 Claims. (Cl. 148—31)

The present invention relates to heat treated and hardened articles of manufacture, and more particularly, to heat treated hardened steel articles of manufacture characterized by a fine grained and normal structure combined with deep hardness and high mechanical properties.

Until comparatively recent years it was the opinion of metallurgists that the physical and mechanical properties of steels and other alloys depended solely upon the chemical composition, and that two samples of any metal or alloy having substantially the same chemical composition would exhibit the same properties under the same conditions. Almost two decades ago, however, it was observed in connection with the carburization of steel that anomalous results in hardening were obtained with steels, which results could not be explained on the basis of differences in amounts of the elements listed in the chemical specifications. McQuaid and Ehn (Transactions A. I. M. E., vol LXVII, 1922, pages 341 et seq.) observed that steels which hardened uniformly and deeply, and which they denoted "normal," were coarse grained, whereas those which were not hardened, or which did not harden uniformly, which they denoted "abnormal," were fine grained. By coarse and fine grained steels, they referred to the austenite grain size as obtained when heated at ordinary carburization temperatures, for example, when subjected to the present A. S. T. M. grain size test, and not to the size of the grains of the steel after cooling to room temperatures. Coarse and fine grained steels are also defined as steels which have low and high coarsening temperatures. Under standard A. S. T. M. grain size test conditions the steels will exhibit fine or coarse grains depending upon whether the coarsening temperature of the particular steel is above or below the temperature used in the test and upon the difference in temperature between the coarsening temperature and the test temperature. Subsequent investigation revealed notable differences in the metallurgical constitution of the normal and the abnormal steels. Davenport and Bain, in their article entitled "General relations between grain size and hardenability and the normality of steels," published in Transactions A. S. M., vol. XXII, 1934, pages 879 et seq., state that normal structure is characterized by "thin, smooth, carbide envelopes entirely contiguous with the finer lamellar pearlite," and that abnormal structure is characterized by "thick carbide envelopes with coarse lamellar pearlite, if any, separated from the network, which may be discontinuous, by a wide

band of ferrite sometimes containing large spheroids of carbide." In an earlier article by Bain entitled "Factors affecting the inherent hardenability of steel" appearing in Transactions A. S. S. T., vol. 20, 1932, pages 385 et seq., Bain stresses the fact that, other things being equal, the fine grained austenite transforms more rapidly, appears more abnormal as cooled, and hardens less deeply than the coarse grained austenite. It follows, therefore, that fine grained steels are associated usually with abnormality and shallow hardenability, whereas coarse grained steels are associated with normal structure and deep hardenability for their alloy content.

The observation of the importance of grain size on the properties of steel naturally was followed by numerous attempts to explain the reason for the difference in grain size, and by extensive search to develop methods for its control. It was found that the addition of certain amounts of aluminum yielded fine grained steel whereas the addition of lesser amounts yielded coarse grained steels. However, the instructions proposed by the art for the control of grain size to produce fine or coarse grained steels could not be modified by selecting intermediate amounts of aluminum to produce an intermediate grain size. It was also recognized that as the silicon content of steel increased above the amount present in commercial steels, the steel tended to become coarser grained.

The problem of producing a fine grain deep hardening normal steel capable also of being heat treated to high hardness still confronted the art despite the numerous attempts which have been made to solve this baffling and outstanding problem.

Although many attempts have been made to remedy the aforementioned shortcomings, none as far as we are aware, was entirely successful when carried into practice commercially.

We have discovered that the prior art shortcomings can be avoided and that new and unexpected results can be consistently obtained by incorporating critical and controlled amounts of aluminum and silicon together in steels.

It is an object of the present invention to provide improved heat treated and hardened articles of manufacture made of fine grained normal steels combining deep hardness with high tensile properties and ductility.

It is another object of the present invention to provide improved heat treated and deep hardened articles of manufacture made of fine grained low alloyed steels having deep harden-

ability combined with physical properties exceeding that of more highly alloyed and more expensive steels.

It is a further object of the present invention to provide heat treated and hardened steel articles of manufacture having a more controllable and predictable grain size.

The invention contemplates the production of heat treated and hardened articles of manufacture made of steels having improved deep hardenability combined with fine grain size, for example, about No. 5 A. S. T. M. or smaller.

The invention also contemplates providing means for converting steels which would ordinarily be coarse grained into fine grained normal steels possessing deep hardening properties.

The invention further contemplates providing means for securing grain sizes within the range of No. 4 to No. 6 A. S. T. M. which heretofore it has been very difficult to obtain consistently.

Other objects of the invention will become apparent to those skilled in the art from the following description taken in conjunction with the accompanying drawings in which:

Fig. 1 is a graph illustrating the effect of aluminum upon the grain size of steel having a normal silicon content;

Fig. 2 is a graph showing the combined effect of aluminum and silicon on the grain size of a low alloyed steel;

Fig. 3 depicts a graph illustrating the combined effect of aluminum and silicon on the hardenability of the same steel;

Fig. 4 is a graph illustrating the effect of aluminum and silicon together upon the hardenability of steel;

Fig. 5 is a series of curves depicting the effect of silicon at various aluminum levels upon the hardenability of a low alloyed steel; and

Fig. 6 shows the depth hardening curves for a steel made in accordance with the present invention and a similar steel containing normal and usual amounts of aluminum and silicon.

We have made a surprising discovery that additional amounts of aluminum above the amounts normally used to control grain size, for example about 0.03%, added to a well deoxidized melt result in the reversal of the aluminum effect on grain size and produce coarsening in grain size, particularly when the aluminum content reaches about 0.08%. The effect of aluminum will be readily observed from Fig. 1 in which the aluminum content is plotted against the grain size of the steel. Typical data illustrative of the reversal in the aluminum effect upon a steel of the S. A. E. 3045 type are included in Table 1:

Table 1

| Steel No. | Nickel   | Chromium | Carbon   | Aluminum | Grain size A. S. T. M. |
|-----------|----------|----------|----------|----------|------------------------|
| 1.        | Per cent | Per cent | Per cent | Per cent | Per cent               |
| 1.-----   | 0.50     | 0.50     | 0.38     | 0        | 1-2                    |
| 2.-----   | 0.50     | 0.49     | 0.41     | 0.03     | 8                      |
| 3.-----   | 0.55     | 0.48     | 0.42     | 0.04     | 7-8                    |
| 4.-----   | 0.50     | 0.53     | 0.39     | 0.05     | 6                      |
| 5.-----   | 0.50     | 0.52     | 0.39     | 0.08     | 5                      |
| 6.-----   | 0.50     | 0.50     | 0.42     | 0.30     | 4                      |
| 7.-----   | 0.50     | 0.50     | 0.36     | 1.00     | 2-4                    |

It will be apparent from Fig. 1 and Table 1 that when aluminum is present in solution in excess of the amount necessary to produce maximum grain refining, i. e., on the descending side of the curve, small amounts of aluminum do not have the large effects on the grain size that is obtained upon the ascending side of the curve. Aluminum

in excess of the amount necessary to produce maximum grain refinement affords greater accuracy in controlling and predicting grain size and for obtaining the desired intermediate grain sizes. Once maximum grain refinement has been reached, change in grain size is markedly slower and more predictable with the resulting wider control over grain size. We have made the further surprising and unexpected discovery that the co-presence of silicon in amounts larger than normal along with aluminum has a marked effect upon the slope of the descending side of the curve and a very strong beneficial effect upon the grain size and the properties of the steel, including hardenability, tensile properties, ductility, impact, etc. Increased amounts of silicon decrease the slope of the curve shown in Fig. 1 on the descending side as well as raise the grain size number obtainable and permit more accurate control of the grain size, particularly in the more useful intermediate grain sizes, than has been possible heretofore. Either silicon or aluminum used alone in sufficient quantity will produce a coarse grain steel whereas the use of the two elements together in amounts that would ordinarily cause grain coarsening if used singly surprisingly results invariably in a fine grain normal steel. When we refer in the specification and claims to "fine grain," "coarse grain," "grain size," the A. S. T. M. grain size number, etc., we mean the austenite grain size as determined under standard test conditions and not the actual grain size. As pointed out by Grossman (Trans. American Soc. for Metals, vol. 22, 1934, p. 861), the austenite grain size is a record of the size of the austenite crystals which existed at high temperatures. Likewise, when we refer to "normal" and "abnormal" structures, we mean the structure as determined under standard test conditions. Both grain size and normality or abnormality usually have been determined by microscopic examination of samples of steel after a specified carburizing cycle which usually would not be employed in commercial practice in ordinary hardening of steels and articles made therefrom. The marked refining effects upon the grain size and the control over grain size of co-present controlled amounts of aluminum and silicon is illustrated in Fig. 2 on S. A. E. 3045 steels. It will be noted from the curves that the reversal effect of aluminum is modified by the co-presence of silicon and that increasing amounts of silicon above normal amounts decrease the grain size for any given aluminum content and also markedly eliminate the possibility of obtaining deleterious coarse grains. Thus at the 0.55% silicon level the grain size is never coarser than about No. 6 (A. S. T. M.) or smaller whereas at the 0.30% silicon level the grain size may be as large as No. 5 or somewhat coarser. Furthermore, increasing amounts of silicon decrease the slope on the descending side of the curve and thereby greatly increase the range of aluminum available for grain size control particularly at the lower aluminum levels where accurate control is most difficult.

The relatively small combined amounts of aluminum and silicon in addition to advantageously affecting grain size, also greatly increase the depth of hardenability of steel whereas aluminum alone in usual amounts produces shallow hardening. The unexpected and highly beneficial effect of co-present and controlled proportions of aluminum and silicon on the hardenability of steel is illustrated in Fig. 3 in which

the surface hardnesses of S. A. E. 3045 steels are plotted against aluminum content for 2.75 inches sections of steels containing 0.30% and 0.55% silicon. It will be noted that the reversal effect of aluminum is present in the hardness curves as well as in the grain size curves and that increasing amounts of silicon gradually eliminate the low hardness areas, i. e., tend to produce uniform hardness at substantially all aluminum levels while markedly increasing the hardness of the steel at all values of aluminum. Similar effects are also obtained at the center of the sections as well as at the surface. Co-present amounts of aluminum and silicon have marked beneficial effects upon both grain size and hardenability and convert steels which would ordinarily be coarse grained into fine grained normal steels while at the same time greatly increasing the hardenability of the steels. The co-presence of controlled amounts of aluminum and silicon effect a more marked increase in the hardenability and the mechanical properties of lower alloyed steels than when they are co-present in highly alloyed intrinsically deep hardening steels. Fig. 4 is a graph showing the effect of co-present amounts of aluminum and silicon, in accordance with the present discovery, upon the hardenability of increasing alloyed steels. The effect of aluminum and silicon on hardenability is most pronounced upon steels of intermediate hardenability whereas the effect on grain size is present regardless of the alloyed content. A very important advantage of the new combination of aluminum and silicon for securing deep hardening is that this property is obtained at less cost than by any known alternative means. By "hardenability" we mean the ability of a steel to harden effectively upon rapidly cooling, e. g., oil quenching, throughout large sections such as two inch sections or larger to approach the hardness obtained in small sections such as one inch sections or smaller. Hardenability is also defined as the ability of a steel to produce a high degree of surface and center hardness in large sections or as the ability of a steel to exhibit complete martensitization. Deep hardening or deep hardenability is defined as the ability of a steel to produce a high surface hardness, for example about 450 Brinell hardness, or higher combined with depth of penetration of that hardness or small change in hardness with penetration. Of course, it will be understood that these characteristics refer to the as quenched condition and that the steels may subsequently be tempered or drawn to lower hardness, for example 350 Brinell hardness, or that the steels may be subjected to an austempering treatment.

Steels containing aluminum and silicon together will thus combine markedly improved deep hardenability and high mechanical properties with low cost, more accurate and reliable grain size, fine grain size and normality as distinguished from abnormality which was heretofore generally characteristic of fine grain aluminum-treated steels.

Broadly stated, the present invention provides improved heat treated and hardened articles of manufacture made of worked steel containing controlled and critical proportions of aluminum and silicon in amounts higher than ordinarily present in steel. The co-presence of aluminum and silicon imparts to the hardened articles accurate grain size, for example, No. 5 (A. S. T. M.) or smaller, and normality to a high degree combined with improved deep hardening character-

istics. The hardened articles also possess markedly increased mechanical properties, including tensile properties, ductility, impact, etc. The pronounced improvement in hardenability is particularly evident in the steels of intermediate alloy content which would in the absence of high silicon and aluminum possess mediocre hardenability. In accordance with the present invention the aluminum and silicon must be controlled within the ranges given in Table II:

Table II

| Element          | Percentage                                |
|------------------|-------------------------------------------|
| 15 Aluminum..... | More than 0.05% but less than about 0.5%. |
| Silicon.....     | More than 0.30% but less than about 0.7%. |

The aluminum amounts given herein are for soluble aluminum as distinguished from aluminum present as aluminum oxide (alumina) which frequently amounts to about 0.06% aluminum as aluminum oxide depending upon the state of deoxidation of the melt at the time of the aluminum addition. The carbon content will ordinarily range between about 0.35% and about 1% carbon. Steels for direct hardening will contain 0.35% to about 0.7% carbon while carburizing steels made in accordance with the present invention although initially containing less than about 0.35% carbon will possess in the carburized condition high properties, including high hardness, at and near the surface where these characteristics are of controlling importance. The manganese content should be at least 0.4%, preferably higher, for example 0.8%. It will be understood that the upper and lower limits stated for silicon and aluminum will vary somewhat with the base composition of the steel and the size of the section. Increased amounts of nickel, manganese and carbon, particularly the latter, will raise the upper limit, whereas such elements as molybdenum and chromium will decrease the upper limit. These opposing effects are believed due to the fact that the first group of elements tend to increase the austenite domain whereas the second group, like aluminum and silicon, decrease the austenite domain. To secure full hardening it is essential to so compose the steel as to render it wholly austenitic at the temperature from which it can be quenched during hardening treatment. The present invention is particularly applicable to alloy steels containing singly or in combination nickel, manganese, chromium and molybdenum and particularly to the intermediate alloy steels containing about 1% to about 3% of alloying elements including manganese, but excluding carbon, silicon and aluminum, which in a 0.40% carbon base composition will fail to harden in the center of a two inch round to about 500 Brinell hardness on oil quenching when aluminum and/or silicon are present only in the usual or normal amounts. The benefits of the present invention are also obtained in plain carbon steels. Such steels usually contain small residual amounts of nickel, chromium and the like which appear in the composition and which may be less than about 0.01% of the composition and as low as about 0.001%. Steels containing singly or in combination the following elements which are commonly added for hardening and strengthening reasons are benefited by the co-presence of aluminum and silicon in accordance with the present invention (Table III).

Table III

| Element    | Percentage    |
|------------|---------------|
| Nickel     | 0.001 to 3.5. |
| Manganese  | 0.4 to 2.0.   |
| Chromium   | 0.001 to 1.5. |
| Molybdenum | 0.001 to 0.5. |

Typical examples of the low alloy contents in steels which are markedly benefited by the present invention are given in Table IV which also includes an illustrative example of carbon steels. It is to be noted that where a blank appears in the table it indicates a commercial absence of the element in question but may be present in small amounts such as 0.01% or 0.001%.

Table IV

| S. A. E. number | Nickel   | Chromium  | Manganese | Molybdenum |
|-----------------|----------|-----------|-----------|------------|
|                 | Per cent | Per cent  | Per cent  | Per cent   |
| 3045            | 0.5-0.7  | 0.5-0.7   | 0.8-1.1   |            |
| 3140            | 1-1.5    | 0.45-0.75 | 0.6-0.9   |            |
|                 | 1.0      | 1.0       | 0.6-1.0   |            |
|                 | 1.0      |           | 0.6-1.0   | 0.25       |
| 4140            |          | 0.8-1.1   | 0.6-0.9   | .15-.25    |
| T1340           | 1.0-1.5  |           | 0.6-0.8   |            |
| 1080            |          |           | 1.6-1.9   |            |
|                 |          |           | 0.6-0.9   |            |

It is understood that in the compositions specified herein, small amounts of minor elements and incidental elements such as sulfur, phosphorus, etc., may be included and when the phrase "balance substantially iron" or "balance substantially all iron" is used it is intended to include minor amounts of such elements which may find their way into the composition as a result of commercial steel making practice or which may be intentionally added in amounts and for the purposes for which such elements have sometimes been employed in ferrous alloy compositions.

In carrying the present invention into practice it is preferred to maintain the aluminum and silicon within the approximate ranges given in Table V. When high hardenability and mechanical properties are desired, for example in direct hardened wrought steel articles, it is also highly advantageous to maintain the carbon and manganese within the ranges given. Excellent properties are obtained if in addition about 1% to 2.6% of alloying elements, for example, nickel and chromium, are also present:

Table V

| Element   | Percentage    |
|-----------|---------------|
| Aluminum  | 0.1 to 0.2.   |
| Silicon   | 0.4 to 0.6.   |
| Carbon    | 0.35 to 0.65. |
| Manganese | 0.50 to 1.2.  |

The present invention contemplates heat treated and hardened articles of manufacture made of wrought steels containing controlled amounts of soluble aluminum and silicon in excess of those normally co-present. The full benefits of the invention are only realized when the steels have been worked and are in the heat treated condition. When the term "heat treated" or "heat treating" is employed herein it is used in the ordinary sense, i. e., it indicates that the steel is heated to just above the critical range and rapidly cooled, for example oil quenched, thereby hardening the steel but also includes austempering or the like. In addition to the quench-

ing treatment it is usually desirable but not necessary to draw or temper the steel by heating to some temperature below the critical range. As a typical example, an S. A. E. 3040 steel would be oil quenched from about 1525° to about 1575° F. depending upon the section size and tempered at temperatures up to about 1200° F. depending upon the properties desired. When high hardnesses are of primary importance the steel is usually tempered below about 900° F., for example 300° to 800° F.

We have found that accurate control of aluminum and silicon within the ranges specified herein is of great importance in obtaining the desired results. Below 0.1% soluble aluminum the total hardness and the hardenability of the steel is less marked and below about 0.05% soluble aluminum abnormality usually results. Above about 0.2 soluble aluminum, further improvement in the properties becomes slightly less pronounced until at about 0.5% soluble aluminum the properties fall off again. Below about 0.20% silicon very little improvement in hardenability is obtained particularly for low aluminum contents. Some improvement is obtained by increasing the silicon to 0.25 or 0.27% but it is preferred that the silicon exceed about 0.30%. With 0.30% silicon there is a rather marked improvement in both hardenability and grain size while far better results are obtained with about 0.4% to about 0.6% silicon. Beyond about 0.7% silicon the hardenability is again reduced rapidly, especially if appreciable aluminum is present and carbon and manganese are low. It is to be observed again that the upper limits for aluminum and silicon depend upon the amount and kind of alloying elements present. Fig. 5 shows the importance of maintaining the aluminum contents above the levels commonly present in steel and also emphasizes the desirability for maintaining the silicon content above about 0.3%. The data for Fig. 5 were obtained from steels containing about 0.5% nickel, 0.5% chromium, 0.5% carbon and 0.8% manganese.

In order that those skilled in the art may have a better understanding of the present invention, typical illustrative examples of the compositions contemplated by the present invention together with their A. S. T. M. grain size are given in Table VI:

Table VI

| Steel No. | Nickel   | Chromium | Manganese | Carbon   | Silicon  | Aluminum | Grain size |
|-----------|----------|----------|-----------|----------|----------|----------|------------|
|           | Per cent | Per cent | Per cent  | Per cent | Per cent | Per cent |            |
| 55        |          |          |           |          |          |          |            |
| 8         | 0.7      | 0.7      | 0.8       | 0.5      | 0.30     | 0.10     | 6-7        |
| 9         | 0.7      | 0.72     | 0.80      | 0.51     | 0.46     | 0.10     | 6-7        |
| 10        | 0.7      | 0.7      | 0.8       | 0.5      | 0.55     | 0.10     | 6-7        |
| 11        | 0.7      | 0.72     | 0.84      | 0.47     | 0.58     | 0.054    | 8          |
| 12        | 0.70     | 0.7      | 0.83      | 0.46     | 0.30     | 0.06     | 8          |
| 13        | 0.5      | 0.52     | 0.80      | 0.47     | 0.34     | 0.052    | 7-8        |
| 14        | 0.5      | 0.53     | 0.78      | 0.52     | 0.43     | 0.10     | 7          |
| 15        | 0.52     | 0.5      | 0.81      | 0.49     | 0.59     | 0.10     | 6-7        |
| 16        | 0.50     | 0.50     | 0.95      | 0.41     | 0.44     | 0.15     | 5-6        |
| 17        | 0.50     | 0.50     | 0.90      | 0.37     | 0.58     | 0.15     | 5-6        |
| 18        | 0.50     | 0.50     | 0.80      | 0.45     | 0.55     | 0.19     | 6          |
| 19        | 0.50     | 0.50     | 0.89      | 0.42     | 0.58     | 0.30     | 5-6        |
| 20        | 0.50     | 0.50     | 0.80      | 0.45     | 0.55     | 0.37     | 6          |
| 21        | 0.50     | 0.50     | 0.80      | 0.45     | 0.30     | 0.58     | 5          |
| 22        | 0.50     | 0.50     | 1.21      | 0.41     | 0.30     | 0.15     | 4-5        |
| 23        | 0.50     | 0.50     | 0.97      | 0.38     | 0.71     | 0.30     | 5          |
| 24        | 0.40     | 0.39     | 0.87      | 0.36     | 0.30     | 0.15     | 4-6        |
| 25        | 0.13     | 0.70     | 0.80      | 0.49     | 0.63     | 0.10     | 7          |
| 26        | 0.60     |          | 1.41      | 0.42     | 0.30     | 0.30     | 4-5        |
| 27        | 1.28     | 0.61     | 0.80      | 0.42     | 0.38     | 0.06     | 7-8        |
| 28        | 1.26     | 0.63     | 0.82      | 0.43     | 0.58     | 0.06     | 7          |

Steels containing aluminum and silicon in the amounts contemplated by the present invention also possess an excellent combination of tensile

strength, hardness and ductility. Typical illustrative examples of the mechanical properties developed by the steels contemplated by the present invention are given in Table VII. The tensile properties are for specimens from sections about 1.25 inches in diameter which are oil quenched from about 1525° F. followed by a draw at about 700° F.

Table VII

| Steel | B. H. N. | T. S. | Y. P. | P. L. | % El. | % R. A. | Impact |
|-------|----------|-------|-------|-------|-------|---------|--------|
| 9     | 444      | 223.0 | 201.5 | 192.0 | 10.5  | 41.9    | 12.3   |
| 15    | 454      | 233.0 | 208.0 | 190.5 | 10.5  | 40.7    | 12.3   |
| 16    | 474      | 231.7 | 201.0 | 179.5 | 10.0  | 39.1    | 7.7    |
| 19    | 477      | 236.7 | 205.0 | 189.0 | 10.0  | 40.7    | 6.2    |
| 27    | 460      | 232.3 | 206.0 | 195.8 | 11.0  | 45.4    | 14     |
| 28    | 484      | 243.3 | 214.5 | 204.8 | 11.0  | 39.7    | 13     |

B. H. N. = Brinell hardness number.

T. S. = Tensile strength in thousand pounds per sq. inch.

Y. P. = Yield point in thousand pounds per sq. inch.

P. L. = Proportional limit in thousand pounds per sq. inch.

% El. = Per cent elongation.

% R. A. = Per cent reduction in area.

Impact = Charpy impact in foot-pounds.

Table VIII gives the mechanical properties of steel No. 27 and No. 28 drawn at 1000° F. instead of at 700° F. as in Table VII:

Table VIII

| Steel | B. H. N.* | T. S. | Y. P. | P. L. | % El. | % R. A. | Impact |
|-------|-----------|-------|-------|-------|-------|---------|--------|
| 27    | 321       | 149.0 | 136.5 | 135.0 | 19.0  | 56.0    | 50     |
| 28    | 332       | 156.0 | 142.5 | 138.4 | 18.0  | 56.0    | 41     |

\*See footnote Table VII for key.

Table IX shows the effect of section size (in inches) upon the mechanical properties of steel No. 16. The smaller size was oil quenched from 1525° F. whereas the larger section was oil quenched from 1550° F. Both sections were then drawn at 700° F.

Table IX

| Size | B. H. N.* | T. S. | Y. P. | P. L. | % El. | % R. A. | Impact |
|------|-----------|-------|-------|-------|-------|---------|--------|
| 1.25 | 474       | 231.7 | 201.0 | 179.5 | 10.0  | 39.1    | 7.7    |
| 2.0  | 418       | 195.5 | 180.0 | 170.0 | 11.5  | 42.8    | 19.7   |

\*See footnote Table VII for key.

Table X illustrates the deep hardening qualities of the steels produced in accordance with the present invention. All specimens were 2 inch wrought sections quenched at 1550° F. (not drawn). The Brinell hardness values given are for the indicated distance from the center of the section:

Table X

| Steel No. | B. H. N. at distance from center (inches) |               |               |               |         |
|-----------|-------------------------------------------|---------------|---------------|---------------|---------|
|           | Center                                    | $\frac{1}{4}$ | $\frac{1}{2}$ | $\frac{3}{4}$ | Surface |
| 9         | 591                                       | 589           | 600           | 600           | 600     |
| 15        | 512                                       | 542           | 555           | 562           | 582     |
| 19        | 564                                       | 539           | *555          | 555           | 555     |
| 28        | 555                                       | 555           | 555           | 555           | 555     |

\*At  $\frac{1}{2}$  inches from center of section.

In Fig. 6 hardenability curves are plotted for two inch sections of steel No. 16 containing 0.44% silicon and 0.15% aluminum (curve A) and for a similar steel (0.5% nickel, 0.49% chromium, 0.77% manganese, and 0.41% carbon) containing normal amounts of aluminum and silicon, i. e., 0.03% aluminum and 0.18% silicon (curve B). The improved hardenability and greater

depth hardness of the improved steel over the ordinary steel is obvious.

The co-presence of aluminum and silicon within the ranges contemplated in the present invention imparts deep hardening properties and an unusually high combination of tensile strength, hardness and ductility, particularly when silicon is present in preferred amounts, for example about 0.6%. Aluminum and silicon are particularly beneficial in the larger sections where initial hardness is lowest and/or in the lower alloy content steels which initially have lower hardnesses.

The improvement in the low alloy nickel-chromium steels is particularly noticeable.

Increased silicon for a given aluminum content, for example 0.06% or 0.1% aluminum, increases the depth hardening properties as distinguished from the shallow hardening characteristic of normal silicon and aluminum containing steels.

The effect is particularly marked when silicon is at least about 0.4% S. A. E. 3050 steels containing aluminum and silicon are improved to such an extent that the properties exceed that of higher alloyed steels, e. g., S. A. E. 4140 steels. S. A. E. 3140 steels produced in accordance with the present invention have hardenabilities exceeding standards S. A. E. 4140, 4640 and 4840 steels, and equal to that of standard S. A. E. 3340 steels, particularly in the larger sized sections.

The steels contemplated by the present invention may be produced in the customary manner used in good steel making practice. It is preferred but not necessary that the melt be completely deoxidized with a silicon-containing deoxidizer such as ferro-silicon or silicon-manganese just previous to the alloy additions of aluminum and silicon to leave the required amounts thereof in the solidified metal as this procedure insures high recoveries and control in the solidified steel and produces maximum effects on increased hardenability.

The co-presence of comparatively small amounts of aluminum and silicon in low alloy steels provides deep hardening, fine grained normal steels and makes possible the use of these steels in a large number of applications which previously required more expensive steels. The present invention provides improved heat treated and hardened articles of manufacture made of worked steels characterized by deep hardening and a fine grained normal structure combined with a high combination of tensile strength and ductility. The articles of manufacture provided by the present invention are made of steels containing besides aluminum and silicon as specified hereinbefore about 0.35% to about 1% carbon, about 0.4% up to 2% manganese, about 0.001% up to about 3.5% of metal from the group consisting of nickel, chromium and molybdenum, more than 0.05% and up to 0.5% aluminum, about 0.3% to about 0.7% silicon, and the balance, i. e., more than about 90% of the steel, is iron. The invention is of particular benefit in heat treated and hardened articles of manufacture made of low alloy steels containing about 1% to 3% of combined manganese and metal of the group consisting of nickel, chromium and molybdenum. Since at least about 0.4% will be manganese, up to about 2.6% of the total may be metal of the group consisting of nickel, chromium and molybdenum. Heat treated and hardened articles of manufacture made of steels containing about 0.4% to about 1.25% nickel, about 0.4% to 0.7% chromium, about 0.5% to about 1.2% manganese, and about 0.35%

70  
75

to about 0.65% carbon in addition to aluminum and silicon in the amounts specified hereinbefore are markedly benefited. Although the present invention is of particular benefit in heat treated and hardened articles of manufacture which during processing have been subjected to direct hardening, it is also applicable to heat treated and hardened articles which have been carburized and which accordingly will exhibit in the carburized regions the beneficial effects and improved properties provided by the present invention. The invention is not concerned with conventionally nitrided steel articles and when a "non-nitrided" article is referred to herein we do not intend to include such articles. Specific examples of improved heat treated and hardened articles include machine elements and other hardened parts which are used in the quenched or quenched and drawn condition, such as automotive and machine parts. Heat treated and hardened axles, shafts, crankshafts, connecting rods, king pins, transmission gears, pinions, ring gears, valves, springs, die blocks, dies, headers, piercers, die inserts and the like are typical examples of the hardened machine elements contemplated by the present invention.

Although the present invention has been described in conjunction with preferred embodiments, it is to be understood that modifications and variations may be resorted to without departing from the spirit and scope of the invention, as those skilled in the art will readily understand. Such variations and modifications are considered to be within the purview and scope of the appended claims.

We claim:

1. As a new article of manufacture, a non-nitrided, heat treated and hardened machine element made of wrought steel constituted of a deep hardened and fine grained to intermediate grained structure comprising about 0.35% to 0.65% carbon, 0.5% to 1.2% manganese, 0.4% to 1.25% nickel, 0.4% to 0.7% chromium, 0.1% to 0.2% aluminum, 0.4% to 0.6% silicon, and the balance substantially all iron, said machine element being characterized by a grain size at least

as small as about No. 5 A. S. T. M. and normality under standard test conditions combined with deep hardness and high mechanical properties.

2. As an article of manufacture, a non-nitrided, heat treated and hardened machine element made of wrought steel constituted of a deep hardened and fine grained to intermediate grained structure comprising about 0.35% to 0.65% carbon, 0.5% to 1.2% manganese, 0.4% to 1.25% nickel, 0.4% to 0.7% chromium, more than 0.05% and up to 0.5% aluminum, more than 0.3% and up to 0.7% silicon, and the balance substantially all iron, said machine element being characterized by a grain size of about No. 5 A. S. T. M. or smaller and normality under standard test conditions combined with deep hardness and high mechanical properties.

3. A heat treated and hardened wrought article of manufacture made of non-nitrided steel constituted of a deep hardened and fine grained to intermediate grained structure comprising about 0.35% to 0.65% carbon, 0.5% to 1.2% manganese, 0.4% to 1.25% nickel, 0.4% to 0.7% chromium, 0.1% to about 0.2% aluminum, 0.4% to 0.6% silicon, and the balance substantially all iron, said article being characterized by a grain size at least as small as about No. 5 A. S. T. M. and normality under standard test conditions combined with deep hardness and high mechanical properties.

4. A heat treated and hardened wrought article of manufacture made of non-nitrided nickel steel constituted of a deep hardened and fine grained to intermediate grained structure comprising about 0.35% to 1% carbon, 0.4% to 2% manganese, 0.4% to 3.5% nickel, 0.4% to 1.5% chromium, more than 0.05% and up to 0.5% aluminum, more than 0.3% and up to 0.7% silicon, and the balance substantially all iron, said article being characterized by a grain size at least as small as about No. 5 A. S. T. M. and normality under standard test conditions combined with deep hardness and high mechanical properties.

ALBERT M. TALBOT  
WILLIAM C. MEARNS.